

## UNITED STATES PATENT OFFICE

CYRUS B. WOOD, OF TAKOMA PARK, DISTRICT OF COLUMBIA

## BLEACHING COMPOUND

No Drawing.

Application filed February 12, 1932. Serial No. 592,662.

(GRANTED UNDER THE ACT OF MARCH 3, 1883, AS AMENDED APRIL 30, 1928; 370 O. G. 757)

This invention described herein may be manufactured and used by or for the Government for governmental purposes without the payment to me of any royalty thereon.

5 This invention relates to a compound for bleaching textiles such as cotton cloth, wool yarn, rayon cloth and the like, and to novel solutions thereof for bleaching purposes.

10 It has been found by the applicant that chloroimide of succinic acid, also known as succinchlorimide, has efficient and advantageous bleaching properties.

This compound is represented by the following structural formula:



The object of this invention is to provide 20 a bleaching agent having an intensity of action which is quite definitely intermediate between the more intense and the less intense bleaching agents heretofore used.

Further objects will be apparent from the 25 following description of the invention.

Broadly the invention comprises the bleaching of textiles and the like by aqueous solutions of succinchlorimide which may be either acid or alkaline in reaction.

30 The bleaching agents at present employed in the textile industry are of various kinds, such as chlorine gas that may be led into watery solutions giving chlorine water, which is a rather active bleaching agent; or the chlorine gas may be led into aqueous solu-

35 tions of sodium carbonate or sodium hydroxide, which results in solutions of more active bleaching agents as they doubtless contain the compound sodium hypochlorite, NaOCl. The chlorine gas may also be allowed to pass over calcium hydroxide with which it reacts, forming chiefly the compound calcium chloro-hypochlorite, ClCaOCl; this product is incompletely soluble in water and such solutions are active bleaching agents.

40 For certain uses in the textile industry bleaching agents are employed which are more mild in their bleaching action than any 45 of the chlorine bleaches disclosed above. Of

this class may be mentioned those of the general type of hydrogen peroxide. In order that alkaline reaction may be established, which is often necessary in bleaching processes, the compound sodium peroxide, Na<sub>2</sub>O<sub>2</sub>, 55 and sodium perborate, NaBO<sub>3</sub>, are also used in the industry.

Bleaching agents are needed for certain purposes in the textile industry which are less prompt and less intense than are the bleaching agents containing chlorine and yet more active than the bleaching agents which are as slow in their bleaching action as those of the general type of hydrogen peroxide or those bleaching processes where alkaline reaction is necessary to be established by using compounds such as sodium peroxide, Na<sub>2</sub>O<sub>2</sub>, or sodium perborate, NaBO<sub>3</sub>.

The new solutions of succinchlorimide have been found to have an intensity for bleaching cotton cloth and the like intermediate between the intensity of the bleaching agents heretofore used.

An acid or alkaline solution of succinchlorimide will also effect bleaching. An aqueous solution of this compound is moderately acid in reaction. There can be added to such solutions certain alkalies; the bleaching properties of acid or alkaline solutions of succinchlorimide being present in about the same 80 relative intensities. Either the acid or alkaline solutions of the succinchlorimide are quite definitely intermediate between the more intense bleaching powder and the less intense sodium perborate.

85 It has been found that cotton cloth may be effectively bleached by the use of an aqueous solution containing 3% of succinchlorimide, which is equivalent to about 1.6% "available chlorine". Weaker solutions of succinchlorimide may of course be used and in some cases are more advantageous. When an alkaline bleaching solution is desired the addition of one equivalent of an alkaline compound to the solution has been found to be effective. For example: four-tenths gram of sodium carbonate may be added to the solution for each gram of succinchlorimide.

90 Having described my invention what I 95 wish to secure by Letters Patent is:

1. A method of bleaching textile materials which comprises subjecting the materials to the action of an aqueous solution of succin-chlorimide.
- 5 2. A method of bleaching textile materials which comprises subjecting the materials to the action of an acid solution of succinchlorimide.
3. A method of bleaching textile materials which comprises subjecting the materials to the action of an alkaline solution of succin-chlorimide.
- 10 4. A composition for bleaching textile material consisting of aqueous solutions of suc-chlorimide.
- 15 5. A composition for bleaching textile material consisting of acid solutions of succin-chlorimide.
- 20 6. A composition for bleaching textile material consisting of alkaline solutions of suc-chlorimide.

CYRUS B. WOOD.